

# UNITED STATES PATENT OFFICE.

HANS GOLDSCHMIDT AND OTTO WEIL, OF ESSEN-ON-THE-RUHR, GERMANY, ASSIGNEES  
TO THE FIRM OF TH. GOLDSCHMIDT, OF ESSEN-ON-THE-RUHR, GERMANY, COM-  
POSED OF KARL GOLDSCHMIDT AND HANS GOLDSCHMIDT.

## METHOD OF RAISING THE ALLOYING QUALIFICATION OF TITANIUM.

1,075,782.

Specification of Letters Patent.

Patented Oct. 14, 1913.

No Drawing.

Application filed October 19, 1910. Serial No. 587,857.

*To all whom it may concern:*

Be it known that we, HANS GOLDSCHMIDT and OTTO WEIL, subjects of the King of Prussia, German Emperor, and residents of Essen-on-the-Ruhr, in the Province of the Rhine, German Empire, have jointly invented certain new and useful Improvements in the Method of Raising the Alloying Qualification of Titanium, of which the following is a specification.

Numerous experiments have shown that it is possible by an addition of titanium to improve considerably the quality of steel and cast-iron. The addition of titanium in a metallic state has been attempted, but on account of the bad alloying qualification, the high melting point and the small specific weight of this metal, the results obtained from such attempts have been entirely unsatisfactory, and because of this experts have been of opinion that in order to obtain good results it is necessary to make use, instead of pure titanium, of an iron-titanium alloy containing only from 10% to 15% of titanium. In many cases, however, it would have been preferable, to add an iron-titanium alloy containing a high percentage of titanium, but the same objections have been raised to the use of such an alloy as to the employment of metallic titanium, the objection in each case being to the use of a high percentage of titanium.

As a result of our experiments we have found that an alloy containing a higher percentage of titanium than has been employed heretofore may be used to advantage in baths of steel and cast-iron if aluminum is added as a third element so that a conjoint action of the titanium alloy and the aluminum takes place in the baths, in which case we, preferably, employ an iron-titanium-aluminum alloy. By using such an alloy as this, with a higher percentage of titanium than has heretofore been employed, the purification of metallic baths, such for example as baths of steel or cast-iron, (by fixing the nitrogen and de-oxidizing and

removing the sulfur) is greatly facilitated. The action takes place much more quickly than when an alloy is used containing only 50 from 10% to 15% of titanium. In practice it has been found advisable to use alloys containing from 15% to 35% of titanium and a quantity of aluminum amounting to about 10% of the titanium present, that is to say, 1.5% to 3.5% of aluminum. The alloy may, however, contain a greater percentage of aluminum. One of the principal advantages resulting from the addition of the aluminum is that the melting point of the 60 titanium alloy is lowered while the alloying qualification is considerably increased.

Iron-titanium-aluminum alloys suitable for the purpose herein described and of any desired composition may be easily produced 65 by the alumino-thermic process. These alloys also have the further advantage of being free from carbon. An alloy containing from 24% to 25% of titanium and 3% of aluminum has proved to be very useful.

What we claim is:

1. The method of treating a metallic bath, which consists in subjecting it to the conjoint action of aluminum and an alloy of titanium containing more than 15% of 75 titanium.

2. The method of treating a metallic bath, which consists in subjecting it to the conjoint action of a small percentage of aluminum and an alloy of titanium containing more than 15% of titanium.

3. The method of treating a metallic bath, which consists in subjecting it to the action of an alloy of titanium containing more than 15% of titanium in combination 85 with at least 1.5% of aluminum.

4. A method of treating a bath of iron or steel, which consists in subjecting it to the action of an alloy of titanium with aluminum containing a greater percentage 90 of titanium than aluminum.

5. A method of treating a bath of iron or steel, which consists in subjecting it to the action of an alloy of ferro-titanium

with aluminum containing a greater percentage of titanium than aluminum.

6. A method of treating a bath of iron or steel, which consists in subjecting it to  
5 the action of an alloy of iron, titanium and aluminum containing from 24% to 25% of titanium and about 3% of aluminum.

In witness whereof we have hereunto set our hands in the presence of two witnesses.

HANS GOLDSCHMIDT. [L. S.]  
OTTO WEIL. [L. S.]

In the presence of—  
CHAS. J. WRIGHT,  
ALFRED HENKEL.